

# UNITED STATES PATENT OFFICE.

LOFTUS HARLEY FRANCIS, OF PRINCETON, CALIFORNIA, ASSIGNOR OF ONE-FOURTH TO CHARLES L. DONOHOE AND ONE-FOURTH TO FRANK FREEMAN, OF WILLOW, CALIFORNIA.

## PROCESS OF TREATING LEATHER WITH COAL-TAR.

No. 834,199.

Specification of Letters Patent.

Patented Oct. 23, 1906.

Application filed May 8, 1906. Serial No. 315,832.

*To all whom it may concern:*

Be it known that I, LOFTUS HARLEY FRANCIS, a citizen of the United States, residing at Princeton, in the county of Colusa and State 5 of California, have invented certain new and useful Improvements in Processes of Treating Leather with Coal-Tar; and I do hereby declare the following to be a full, clear, and exact description of the invention, such as 10 will enable others skilled in the art to which it appertains to make and use the same.

This invention, which relates to the preservation of leather, contemplates an improved process of treating this material to obtain 15 the complete saturation or impregnation thereof with coal-tar, whereby the treated leather is without impairment of strength and flexibility rendered absolutely vermin and water proof and its wear-resisting quality is 20 greatly enhanced.

In practicing the improved process I prepare a bath of coal-tar having a temperature of approximately one hundred and ten (110) degrees Fahrenheit and immerse therein 25 leather which has been tanned by the usual method and which may be in a split or un-split condition and either before or after the rolling and glossing steps employed to fit the material as to weight or density, according 30 to its intended use. The leather is kept immersed in the bath at the stated temperature for a period of time ranging from twenty-four (24) hours to six (6) days, dependent upon its density or thickness or the use for 35 which it is intended, during which period it becomes thoroughly saturated or impregnated with the coal-tar. The saturated or impregnated leather is then removed from the bath and is passed between rollers exerting pressure 40 sure to express therefrom the superfluous

coal-tar and to force the retained coal-tar into all of the fibers. The rolled leather is then placed upon drying-racks or the like, and when the moisture is nearly expelled it is again passed between pressure-rollers and 45 when desired is glossed in the usual manner.

The products from different coal-gas or coal-tar works usually vary in weight, and it is advisable in case of heavy tar to add a small quantity of gasolene or the like to reduce the weight and assist absorption, which 50 is accomplished by capillary action.

The absorbed coal-tar is thoroughly incorporated with the fibers of the leather, and in drying the leather becomes a compact gutta- 55 percha-like material having a high wear-resisting quality compared with leather which has not been so treated. Moreover, leather treated by this process retains its strength and flexibility, is antiseptic and vermin- 60 proof, and will not become impaired by long exposure to water.

I claim—

The herein-described process of treating leather with coal-tar, which consists in immersing the same for from one to six days in a bath of coal-tar having a temperature of approximately one hundred and ten degrees Fahrenheit, passing the tanned leather between pressure-rollers, abstracting by drying 65 a portion of the moisture from the rolled leather, and again rolling the partly-dried leather. 70

In testimony whereof I affix my signature in presence of two witnesses.

LOFTUS HARLEY FRANCIS.

Witnesses:

MOLLIE LOHSE,  
CAT. EHOM.